



US011292981B2

(12) **United States Patent**  
**Li et al.**

(10) **Patent No.:** **US 11,292,981 B2**  
(45) **Date of Patent:** **Apr. 5, 2022**

(54) **EMULSIFIER FOR LUBRICATING OIL CONCENTRATE**

(71) Applicant: **Huntsman Petrochemical LLC**, The Woodlands, TX (US)

(72) Inventors: **Xiaolong Li**, Shanghai (CN); **Wei-Yang Su**, Spring, TX (US); **Jun Fan**, Shanghai (CN)

(73) Assignee: **HUNTSMAN Petrochemical LLC**, The Woodlands, TX (US)

(\*) Notice: Subject to any disclaimer, the term of this patent is extended or adjusted under 35 U.S.C. 154(b) by 0 days.

(21) Appl. No.: **16/358,934**

(22) Filed: **Mar. 20, 2019**

(65) **Prior Publication Data**

US 2019/0218469 A1 Jul. 18, 2019

**Related U.S. Application Data**

(63) Continuation of application No. 14/363,355, filed as application No. PCT/CN2012/077577 on Jun. 27, 2012, now abandoned.

(51) **Int. Cl.**

**C10M 133/08** (2006.01)  
**C10M 173/00** (2006.01)  
**C10N 30/12** (2006.01)  
**C10N 30/18** (2006.01)  
**C10N 30/00** (2006.01)  
**C10N 40/20** (2006.01)  
**C10N 70/00** (2006.01)

(52) **U.S. Cl.**

CPC ..... **C10M 133/08** (2013.01); **C10M 173/00** (2013.01); **C10M 2201/087** (2013.01); **C10M 2203/1006** (2013.01); **C10M 2203/1025** (2013.01); **C10M 2203/1045** (2013.01); **C10M 2203/1065** (2013.01); **C10M 2203/1085** (2013.01); **C10M 2207/126** (2013.01); **C10M 2207/40** (2013.01); **C10M 2215/04** (2013.01); **C10M 2215/042** (2013.01); **C10M 2219/044** (2013.01); **C10N 2030/12** (2013.01); **C10N 2030/18** (2013.01); **C10N 2030/24** (2020.05); **C10N 2040/20** (2013.01); **C10N 2070/02** (2020.05)

(58) **Field of Classification Search**

CPC ..... C10M 133/08; C10M 173/00; C10M 2201/087; C10M 2203/1025; C10M

2203/1045; C10M 2203/1065; C10M 2203/1085; C10M 2207/126; C10M 2207/04; C10M 2215/042; C10M 2219/044

See application file for complete search history.

(56)

**References Cited**

**U.S. PATENT DOCUMENTS**

3,840,611 A \* 10/1974 Gau ..... C07C 7/173  
585/853  
4,118,331 A \* 10/1978 Jahnke ..... C10M 141/10  
508/306  
4,268,404 A \* 5/1981 Ahlgrim ..... C10M 125/24  
508/162  
4,402,844 A \* 9/1983 Trepka ..... C08C 19/42  
508/243  
6,271,185 B1 \* 8/2001 Kodali ..... C10M 105/00  
508/487  
6,548,456 B1 \* 4/2003 Mulder ..... C10M 133/44  
508/268  
6,617,303 B1 \* 9/2003 Smith ..... C11D 1/44  
510/336  
2006/0270569 A1 \* 11/2006 Athans ..... C10M 173/00  
508/491  
2010/0093868 A1 \* 4/2010 Kadokawa ..... A01N 33/04  
514/671  
2010/0222618 A1 \* 9/2010 Takagi ..... C10M 105/04  
585/1

**OTHER PUBLICATIONS**

Huntsman Performance Products Metalworking Chemicals, Americas Product Information Brochure, retrieved from the internet at <[http://web.archive.org/web/20081204095243/http://www.huntsman.com/performance\\_products/Media/MW\\_Americas\\_Product\\_Information.pdf](http://web.archive.org/web/20081204095243/http://www.huntsman.com/performance_products/Media/MW_Americas_Product_Information.pdf)> on Aug. 15, 2019 (Year: 2008).\*

\* cited by examiner

*Primary Examiner* — James C Goloboy

(74) *Attorney, Agent, or Firm* — Huntsman Petrochemical LLC; Aleece M. Hayes

(57)

**ABSTRACT**

The present disclosure provides a lubricating oil concentrate containing an ethoxylated ether amine and a base oil. The lubricating oil concentrate is capable of forming a stable, low foaming emulsion when added to an aqueous medium and may be useful in metalworking and cleaning fluids.

**8 Claims, No Drawings**



aqueous medium, produces an aqueous emulsion that exhibits improved stability, good wetting and low foaming properties while also being environmentally friendly.

According to one embodiment, the ethoxylated ether amine is a compound represented by the formula (I)



where R=a straight chain or branched alkyl group having from 8 to 22 carbon atoms;

n=an integer from 2 to 30;

x=an integer from 1 to 29; and

y=an integer from 1 to 30.

In one embodiment, the ethoxylated ether amine is a compound represented by the formula (I) where R=a straight chain or branched alkyl group having from 10 to 18 carbon atoms, preferably from 12 to 16 carbon atoms.

In another embodiment, the ethoxylated ether amine is a compound represented by the formula (I) where R=a straight chain or branched alkyl group having from 8 to 22 carbon atoms, preferably from 12 to 16 carbon atoms.

In still another embodiment, the ethoxylated ether amine is a compound represented by the formula (I) where R=a straight chain or branched alkyl group having from 10 to 18 carbon atoms, preferably from 12 to 16 carbon atoms.

In some embodiments, the ethoxylated ether amine of formula (I) may be present in the oil concentrate in an amount of about 1% by weight to about 90% by weight, based on the total weight of the oil concentrate. In another embodiment, the ethoxylated ether amine of formula (I) may be present in the oil concentrate in an amount of about 2% by weight to about 50% by weight, based on the total weight of the oil concentrate. In still another embodiment, the ethoxylated ether amine of formula (I) may be present in the oil concentrate in an amount of about 5% by weight to about 20% by weight, based on the total weight of the oil concentrate.

The oil concentrate of the present disclosure also includes a base oil. In some embodiments, the base oil will have a kinematic viscosity in the range of from about 1 cSt to about 1000 cSt at a temperature of 40° C. In one particular embodiment, the base oil is a petroleum-based oil, vegetable oil, animal-derived oil or synthetic oil.

Examples of petroleum-based oils which may be used in the present disclosure include, but are not limited to, naphthalenic oils, paraffinic oils, crude oils, diesel oils, mineral seal oils, kerosenes, fuel oils, white oils and aromatic oils.

Examples of vegetable oils or animal-derived oils include, but are not limited to, canola oil, walnut oil, cashew nut oil, olive oil, corn oil, peanut oil, grape seed oil, oiticica oil, palm oil, rapeseed oil, fish oil, fish liver oil, sperm oil, oleic acid, bear oil, whale oil, and linseed oil.

Examples of synthetic oils include, but are not limited to, hydrocarbon oils and halo-substituted hydrocarbon oils such as polymerized and interpolymerized olefins, for example polybutylenes, polypropylenes, propylene-isobutylene copolymers, chlorinated polybutylenes, poly(1-hexenes), poly(1-octenes), poly(1-decenes); alkyl benzenes, such as dodecylbenzenes, tetradecylbenzenes, dinonylbenzenes, di-

(2-ethylhexyl)benzenes; polyphenyls such as biphenyls, terphenyls, and alkylated polyphenyls; and alkylated diphenyl ethers and alkylated diphenyl sulfides and derivatives, analogs and homologs thereof. Alkylene oxide polymers and derivatives thereof where terminal hydroxy groups have been modified by esterification, etherification etc. constitute another class of synthetic oils. These are exemplified by polyoxyalkylene polymers prepared by the polymerization of ethylene oxide or propylene oxide, the alkyl and aryl ethers of these polyoxyalkylene polymers such as methylpolyisopropylene glycol ethers, diphenyl and diethyl ethers of polyethylene glycol; and mono and polycarboxylic esters thereof, for example, the acetic esters, mixed C<sub>3</sub>-C<sub>8</sub> aliphatic acid esters, C<sub>12</sub>-C<sub>22</sub> fatty acid esters, and C<sub>13</sub> oxo diester of tetraethylene glycol. Simple aliphatic ethers may be used as synthetic oils, such as, diethyl ether, didecyl ether, di(2-ethylhexyl) ether. Other synthetic oils comprise the esters of fatty acids such as ethyl oleate, lauryl hexanoate, and decyl palmitate and the esters of dicarboxylic acids such as phthalic acid, succinic acid, maleic acid, azelaic acid, sebacic acid, fumaric acid, adipic acid, linoleic acid dimer, malonic acid, alkyl malonic acids, alkene malonic acids with a variety of alcohols such as butyl alcohol, hexyl alcohol, dodecyl alcohol, 2-ethylhexyl alcohol, ethylene glycol, diethylene glycol monoethyl ether, propylene glycol are also useful. Specific examples of these esters include dibutyl adipate, di(2-ethylhexyl) sebacate, di-n-hexyl fumarate, diethyl sebacate, diisooctyl azelate, diethyl phthalate, didecyl phthalate, dieicosyl sebacate, the 2-ethylhexyl diester of linoleic acid dimer, and the complex ester formed by reacting one mole of sebacic acid with two moles of tetraethylene glycol and two moles of 2-ethyl-hexanoic acid. and polyalphaolefins.

In still another embodiment, the base oil is a mixture of at least two of the oils described above.

According to some embodiments, the base oil may be present in the oil concentrate in an amount of about 0.5% by weight to about 97.5% by weight, based on the total weight of the oil concentrate. In another embodiment, the base oil may be present in the oil concentrate in an amount of about 5% by weight to about 95% by weight, based on the total weight of the oil concentrate. In other embodiments, the base oil is present in the oil concentrate in an amount greater than about 40% by weight, based on the total weight of the oil concentrate. In further embodiments, the base oil is present in the oil concentrate in an amount less than about 40% by weight, based on the total weight of the oil concentrate. In still other embodiments, the base oil is present in the oil concentrate in an amount of about 30% by weight to about 85% by weight, based on the total weight of the oil concentrate while in other embodiments, the base oil is present in the oil concentrate in an amount of about 5% by weight to about 30% by weight, based on the total weight of the oil concentrate.

55 Optionally, the water-miscible lubricating oil concentrate may contain one or more additives. Such additives include, but are not limited to: corrosion inhibitors, such as alkaline and alkanolamine salts of organic acids, sulfonates, amines, amides, and organic borate compounds; biocides, such as o-phenylphenol; bactericides, fungicides and algaecides; colorants; fragrances; surfactants; chelating agents; pH buffering agents; solubilizers, anti-oxidants; anti-foaming agents; extreme pressure agents; and mixtures thereof.

The water-miscible lubricating oil concentrate may be prepared by admixing the ethoxylated ether amine with the base oil such that upon its addition to an aqueous medium, for example water, a stable, low foaming aqueous emulsion

results. The water-miscible lubricating oil concentrate may be used "as-is" or may be diluted with water or other aqueous solution prior to addition to the aqueous medium. Thus, in another embodiment, water is added to the water-miscible oil concentrate to dilute the oil concentrate of the present disclosure and the oil concentrate is then added to the aqueous medium to form a stable, low foaming aqueous emulsion. In a further embodiment, the water and/or aqueous medium is deionized water.

As noted above, the water-miscible lubricating oil concentrate of the present disclosure, upon addition to an aqueous medium, forms a stable, low foaming aqueous emulsion which may be used in many applications, such as metalworking fluids for metalworking processes. In addition, the aqueous emulsion exhibits surprisingly good wetting properties and non ferrous metal protection and may also be used in cleaning fluids. Aqueous emulsions of the oil-in-water and water-in-oil type may be formed with the addition of from about 1 weight part to about 40 weight parts, preferably from about 2 weight parts to about 30 weight parts, and more preferably from about 5 weight parts to about 20 weight parts of lubricating oil concentrate per 100 weight parts of aqueous medium. In most embodiments, the aqueous medium is water, preferably deionized water.

Thus, in another embodiment, there is provided a metalworking or cleaning fluid comprising an aqueous emulsion wherein the aqueous emulsion includes an oil phase dispersed in a continuous aqueous medium, the oil phase containing the lubricating oil concentrate and the aqueous medium containing water.

Metalworking processes where the metalworking fluid may be used include, but are not limited to, elastic deformation, plastic deformation and cold working of metals, with or without metal removal. In some of these operations the metal piece is deformed only; like in rolling, drawing, stamping, forging and blanking of steel and aluminum, while in others metal is removed rather than deformed, like in cutting, grinding, turning, milling, tapping, broaching, machining and drilling of metals. The metallic material from which the metalworking apparatus and articles to be fabricated are made, include steel, cast iron, and ferrous alloys, as well as aluminum alloys and other non-ferrous alloys, including such components as titanium, magnesium, copper, tin and brass.

In one particular embodiment, the water-miscible lubricating oil concentrate may be used in a cutting process. A lubricating oil concentrate formulation dispersed in an aqueous medium at a concentration of about 5 weight parts to 20 weight parts of oil concentrate per 100 weight parts of aqueous medium (for e.g. water) may include the following:

| Oil Concentrate Components | Wt. % based on the total weight of oil concentrate |
|----------------------------|----------------------------------------------------|
| Paraffinic Oil             | 60 to 70                                           |
| Ethoxylated ether amine    | 10 to 18                                           |
| Diglycolamine              | 3 to 6                                             |
| Inorganic Acid             | 1 to 4                                             |
| Organic Acid               | 1 to 2                                             |
| Stabilizer                 | 2 to 4                                             |
| Tall Oil Fatty Acid        | 6 to 10                                            |
| Deionized Water            | 0.5 to 3                                           |

In another embodiment, the water-miscible lubricating oil concentrate may be used for an aluminum cutting or grinding process. A lubricating oil concentrate formulation for an aluminum cutting or grinding process dispersed in an aqueous

medium at a concentration of about 5 weight parts to about 20 weight parts of oil concentrate per 100 parts of aqueous medium (for e.g. water) may include the following:

| Oil Concentrate Components | Wt. % based on the total weight of the oil concentrate |
|----------------------------|--------------------------------------------------------|
| Paraffinic Oil             | 10 to 20                                               |
| Ethoxylated ether amine    | 10 to 20                                               |
| Nonionic Surfactants       | 5 to 15                                                |
| Tall Oil                   | 6 to 10                                                |
| Stabilizer                 | 1 to 3                                                 |
| Diglycolamine              | 5 to 10                                                |
| Inorganic Acid             | 3 to 5                                                 |
| Organic Acid               | 1 to 3                                                 |
| Amine                      | 0.2 to 0.6                                             |
| Deionized Water            | Balance to 100                                         |

The following examples are provided to illustrate embodiments of the present disclosure but are not intended to limit the scope thereof.

#### Example 1

Emulsifying properties and foam resistance were evaluated for four different commercially available sodium sulfonate (M, H, HL, and L) emulsifiers and an ethoxylated ether amine according to the present disclosure (Surfonic® PEA-25 emulsifier available from Huntsman Petrochemical LLC). The oil concentrates were prepared by adding each emulsifier at various dosages (5 wt. %, 8 wt. %, and 12 wt. % of emulsifier, based on the total weight of the oil concentrate) to a base oil (paraffin-base oil).

5.0 grams of the resulting oil concentrate and 95.0 grams of deionized water were then added to a graduated cylinder. The cylinder was stoppered, shook, and various properties were then measured. The results are given below in Table 1 through 3.

#### Materials Used for Example 1

| Emulsifier       | Sodium Sulfonate   |                |                |                |
|------------------|--------------------|----------------|----------------|----------------|
| Material         | Aristonate ® M     | Aristonate ® H | Petronate ® HL | Petronate ® L  |
| Name             | M                  | H              | HL             | L              |
| Average          | 430                | 460            | 450            | 420            |
| Molecular Weight |                    |                |                |                |
| Material Type    | Synthetic          |                |                |                |
| Supplier         | Pilot Chemical Co. |                | Natural        | Sonneborn Inc. |

  

| Paraffin-base oil                      |                                  |  |  |  |
|----------------------------------------|----------------------------------|--|--|--|
| Material Name                          | HVI 1a 150 (150N Paraffinic Oil) |  |  |  |
| Viscosity (40° C.), mm <sup>2</sup> /s | 28.00-32.00                      |  |  |  |
| Supplier                               | Sinopec                          |  |  |  |

TABLE 1

| Performance Comparison with Emulsifier Dosage at 5 wt % |             |    |    |    |    |
|---------------------------------------------------------|-------------|----|----|----|----|
|                                                         | Formulation |    |    |    |    |
|                                                         | A           | B  | C  | D  | E  |
| Material 150SN                                          | 95          | 95 | 95 | 95 | 95 |
| PEA 25                                                  | 5           |    |    |    |    |
| M                                                       |             | 5  |    |    |    |
| H                                                       |             |    | 5  |    |    |
| HL                                                      |             |    |    | 5  |    |
| L                                                       |             |    |    |    | 5  |

  

| Test Results                             |                     |     |     |     |                    |
|------------------------------------------|---------------------|-----|-----|-----|--------------------|
|                                          | Foam Resistance(cm) |     |     |     |                    |
| Start                                    | 4.3                 | 8.5 | 9.0 | 5.8 | 6.5                |
| 5 min later                              | 3.0                 | 8.0 | 8.5 | 5.0 | 6.0                |
| Emulsifying Properties, Cream Volume, ml |                     |     |     |     |                    |
| 3 min                                    | 1.5                 | 6.0 | 8.5 | 7.0 | 1.5/4.5(Oil/Cream) |
| 15 min                                   | 2.0                 | 8.5 | 9.5 | 9.0 | 2.0/5.5(Oil/Cream) |

TABLE 2

| Performance Comparison with Emulsifier Dosage at 8% |             |    |    |    |    |
|-----------------------------------------------------|-------------|----|----|----|----|
|                                                     | Formulation |    |    |    |    |
|                                                     | F           | G  | H  | I  | J  |
| Material 150SN                                      | 92          | 92 | 92 | 92 | 92 |
| PEA 25                                              | 8           |    |    |    |    |
| M                                                   |             | 8  |    |    |    |
| H                                                   |             |    | 8  |    |    |
| HL                                                  |             |    |    | 8  |    |
| L                                                   |             |    |    |    | 8  |

  

| Test Results                             |                     |     |     |     |     |
|------------------------------------------|---------------------|-----|-----|-----|-----|
|                                          | Foam Resistance(cm) |     |     |     |     |
| Start                                    | 4.8                 | 9.0 | 6.5 | 6.8 | 6.5 |
| 5 min later                              | 3.8                 | 8.5 | 6.0 | 6.5 | 6.2 |
| Emulsifying Properties, Cream Volume, ml |                     |     |     |     |     |
| 3 min                                    | 0.2                 | 3.0 | 3.0 | 6.0 | 5.0 |
| 15 min                                   | 1.0                 | 8.0 | 7.5 | 5.0 | 4.5 |

TABLE 3

| Performance Comparison with Emulsifier Dosage at 12% |             |    |    |    |    |
|------------------------------------------------------|-------------|----|----|----|----|
|                                                      | Formulation |    |    |    |    |
|                                                      | K           | L  | M  | N  | O  |
| Material 150SN                                       | 88          | 88 | 88 | 88 | 88 |
| PEA 25                                               | 12          |    |    |    |    |
| M                                                    |             | 12 |    |    |    |
| H                                                    |             |    | 12 |    |    |
| HL                                                   |             |    |    | 12 |    |
| L                                                    |             |    |    |    | 12 |

  

| Test Results                             |                     |     |     |     |     |
|------------------------------------------|---------------------|-----|-----|-----|-----|
|                                          | Foam Resistance(cm) |     |     |     |     |
| Start                                    | 4.5                 | 8.0 | 5.5 | 8.0 | 9.0 |
| 5 min later                              | 3.0                 | 7.0 | 4.5 | 6.5 | 8.5 |
| Emulsifying Properties, Cream Volume, ml |                     |     |     |     |     |
| 3 min                                    | 0.0                 | 1.5 | 2.0 | 0.5 | 0.2 |
| 15 min                                   | 0.1                 | 5.5 | 9.0 | 2.5 | 2.5 |

Example 2

## Soluble Oil Formulation

The following oil concentrate formulation at about 5 weight parts to 10 weight parts per 100 parts of oil concentrate per 100 weight parts water was prepared. The emulsions performance was then measured and the results are provided in Table 4 below:

TABLE 4

| Oil Concentrate Components | Wt. % based on the total weight of oil concentrate |
|----------------------------|----------------------------------------------------|
| 150N Paraffinic Oil        | 65%                                                |
| Diglycolamine              | 4.7%                                               |
| Boric Acid                 | 2.6%                                               |
| Caprylic Acid              | 1.4%                                               |
| Surfonic ® WT-2524         | 3%                                                 |
| Surfonic ® PEA 25          | 14%                                                |
| Tall Oil Fatty Acid        | 8%                                                 |
| Deionized Water            | 1.3%                                               |

  

| Test Results                    |               |
|---------------------------------|---------------|
| Appearance(Concentrate)         | clear         |
| Concentrate Stability           |               |
| High Temp@50° C., 4 H           | clear         |
| Appearance (Emulsion @ 5%)      | Milky white   |
| pH @ 5%                         | 9.05          |
| Emulsion Stability @ 5%, 25° C. | Oil/Cream, ml |
| 200 ppm Hard Water              | none/Trace    |
| 400 ppm Hard Water              | none/0.1      |

## Semi-Synthetic Fluid Formulation

The following oil concentrate at about 5 weight parts to 20 weight parts of oil concentrate per 100 weight parts water provides excellent emulsion stability. No aluminum staining was observed.

| Oil Concentrate Components | Wt. % based on the total weight of the oil concentrate |
|----------------------------|--------------------------------------------------------|
| 150N Paraffinic Oil        | 15%                                                    |
| Surfonic ® PEA 25          | 15%                                                    |
| Surfonic ® L4-2            | 2%                                                     |
| Tall Oil                   | 8%                                                     |
| Surfonic ® WT-2524         | 2%                                                     |
| Diglycolamine              | 7.5%                                                   |
| Boric Acid                 | 4.2%                                                   |
| Caprylic Acid              | 2.3%                                                   |
| Surfonic ® POA-17R2        | 1.6%                                                   |
| Surfonic ® POA-17R4        | 1.6%                                                   |
| Jeffamine ® T-403          | 0.4%                                                   |
| Teric 12A3 Surfactant      | 5%                                                     |
| Deionized Water            | 35.4%                                                  |

  

| Test Results                                                     |               |
|------------------------------------------------------------------|---------------|
| Appearance(Concentrate)                                          | clear         |
| Concentrate Stability                                            |               |
| High Temp@50° C., 4 H                                            | clear         |
| Appearance (Emulsion, 5%)                                        | translucent   |
| pH @ 5%                                                          | 9.42          |
| Emulsion Stability @ 5%, ambient temperature                     | Oil/Cream, ml |
| 200 ppm Hard Water                                               | none/none     |
| 400 ppm Hard Water                                               | none/none     |
| Aluminum Stain Test @ 5% (24 hr immersion, ambient temperature): |               |
| 7075Al                                                           | No stain      |
| 6061Al                                                           | No stain      |

| Oil Concentrate Components                  | Wt. % based on the total weight of the oil concentrate |
|---------------------------------------------|--------------------------------------------------------|
| 3191Al                                      | No stain                                               |
| 2024Al                                      | No stain                                               |
| Rust Protection Test@2%                     |                                                        |
| Chip rust @ rust area %, DI-Water           | 0%                                                     |
| Chip rust @ rust area %, 200 ppm Hard Water | 25%                                                    |

Consideration must be given to the fact that although this disclosure has been described and disclosed in relation to certain preferred embodiments, obvious equivalent modifications and alterations thereof will become apparent to one of ordinary skill in this art upon reading and understanding this specification and the claims appended hereto. The present disclosure includes the subject matter defined by any combination of any one of the various claims appended hereto with any one or more of the remaining claims, including the incorporation of the features and/or limitations of any dependent claim, singly or in combination with features and/or limitations of any one or more of the other dependent claims, with features and/or limitations of any one or more of the independent claims, with the remaining dependent claims in their original text being read and applied to any independent claim so modified. This also includes combination of the features and/or limitations of one or more of the independent claims with the features and/or limitations of another independent claim to arrive at a modified independent claim, with the remaining dependent claims in their original text being read and applied to any independent claim so modified. Accordingly, the presently disclosed invention is intended to cover all such modifications and alterations, and is limited only by the scope of the claims which follow, in view of the foregoing and other contents of this specification.

What is claimed is:

1. An aqueous emulsion consisting of:  
about 5 to about 20 weight parts of a water-miscible lubricating oil concentrate consisting of:  
(i) from about 10% by weight to about 20% by weight, based on the total weight of the water-miscible lubricating oil concentrate, of an ethoxylated ether amine having the formula (I)



where R=a straight chain or branched alkyl group having from 8 to 22 carbon atoms;  
n=an integer from 2 to 30;  
x=an integer from 1 to 29; and  
y=an integer from 1 to 30; and  
(ii) greater than about 40% by weight, based on the total weight of the water-miscible lubricating oil concentrate, of a base oil consisting of a petroleum-based oil and a second petroleum-based oil; and optionally  
(iii) at least one of a corrosion inhibitor, a o-phenylphenol, a colorant, a fragrance, a surfactant, a pH

buffering agent, a solubilizer, an anti-oxidant, an anti-foaming agent, an extreme pressure agent, and water; and

100 weight parts of water.

5 2. The aqueous emulsion of claim 1, wherein R=a straight chain or branched alkyl group having from 12 to 16 carbon atoms.

3. The aqueous emulsion of claim 1, wherein y=an integer from 2 to 6.

10 4. The aqueous emulsion of claim 1, wherein n=an integer from 5 to 20 and x=an integer from 4 to 19.

5. The aqueous emulsion of claim 1, wherein the petroleum-based oil is selected from naphthalenic oil, paraffinic oil, crude oil, diesel oil, mineral seal oil, kerosene, fuel oil, white oil, and aromatic oil.

15 6. The aqueous emulsion of claim 1, wherein the water-miscible lubricating oil concentrate further comprises a surfactant and/or water.

20 7. A method of preparing an aqueous emulsion consisting of:

about 5 to about 20 weight parts of a water-miscible lubricating oil concentrate consisting of admixing about 10% by weight to about 20% by weight, based on the total weight of the water-miscible lubricating oil concentrate, ethoxylated ether amine having the formula (I)



where R=a straight chain or branched alkyl group having from 8 to 22 carbon atoms;

n=an integer from 2 to 30;

x=an integer from 1 to 29; and

y=an integer from 1 to 30, with greater than about 40%

30 by weight, based on the total weight of the water-miscible lubricating oil concentrate, of a base oil consisting of a petroleum-based oil and a second petroleum-based oil, and optionally at least one of a corrosion inhibitor, o-phenylphenol, a colorant, a fragrance, a surfactant, a pH buffering agent, a solubilizer, an anti-oxidant, an anti-foaming agent, an extreme pressure agent, and water; and

100 weight parts of water.

50 8. A metal working or cleaning fluid consisting of an aqueous emulsion wherein the aqueous emulsion consists of an oil phase dispersed in a continuous aqueous medium, the oil phase consisting of about 5 to about 20 weight parts of a water-miscible lubricating oil concentrate of:

55 (i) from about 10% by weight to about 20% by weight, based on the total weight of the water-miscible lubricating oil concentrate, of an ethoxylated ether amine having the formula (I)



60 where R=a straight chain or branched alkyl group having from 8 to 22 carbon atoms;

**11**

n=an integer from 2 to 30;  
x=an integer from 1 to 29; and  
y=an integer from 1 to 30; and  
(ii) greater than about 40% by weight, based on the total  
weight of the water-miscible lubricating oil concen- 5  
trate, of a base oil consisting of a petroleum-based oil  
and a second petroleum-based oil;  
the aqueous medium consisting of 100 weight parts of water.

**12**

\* \* \* \* \*